

# UNITED STATES PATENT OFFICE.

JOHN W. FRIES, OF WINSTON-SALEM, NORTH CAROLINA.

## COMPOSITION FOR USE IN DYEING.

1,266,577.

Specification of Letters Patent.

Patented May 21, 1918.

No Drawing.

Application filed June 16, 1915. Serial No. 34,415.

To all whom it may concern:

Be it known that I, JOHN W. FRIES, a citizen of the United States, and resident of Winston-Salem, county of Forsyth, and

5 State of North Carolina, have invented an Improvement in Compositions for Use in Dyeing, of which the following is a specification.

The object of my invention is to provide 10 a suitable dye composition, preferably in a powdered form, which may be subsequently employed, when properly diluted, to furnish a dyeing solution to which textile material, more particularly cotton or cotton goods, 15 may be treated and thereby dyed with a permanent color of the desired shade.

More particularly, my object is to provide 20 a dye composition employing, as an essential element vegetable dye-stuffs treated in such 25 manner as to provide a composition of the same associated with a metallic hydrated oxid, the said resulting dye composition preferably in a form which may be packed in concentrated condition either as a powder or of a thick syrupy consistency. My object 30 is further to provide a vegetable dye which shall be readily soluble in water and capable of dyeing cotton in one bath such as is possible with the direct anilin dyes; further, in 35 which the color may be developed and deepened by oxidation through exposure to the air during drying; also to provide a vegetable dye of inexpensive character giving 40 highly satisfactory results which does not "bleed", as occurs with direct anilin dyes and which shall therefore be superior to such dyes.

My object is also to provide a suitable dye 45 of the character above stated, which, by using soap or alizarin oil, or similar substances in the dye bath, will permit the cotton to be entered dry with satisfactory results and thereby save the time, trouble and expense of "wetting out", which is usually necessary.

As a rule, the vegetable dye-stuffs heretofore used, are precipitated by metallic salts and the methods used are more or less unsatisfactory, sometimes requiring long boiling 50 and often repeated operations. The dye-woods have been used more particularly for blacks, browns, tans, etc., on cotton, but heretofore they have furnished no satisfactory blue, and it is one of the special objects of my invention to employ logwood as 55 a basis for the production of a composition

capable of producing a most satisfactory blue, not only of one color, but of different shades at the option of the dyer.

In the production of my improved dye 60 composition, I employ dyewood extracts and especially logwood, preferably in the form of a liquid extract, and to this I add an ammoniacal solution of hydrated metallic oxid according to the color or shade to be pro- 65 duced, the mixture being in such proportions and the hydrated metallic oxid formed in such manner that the desired final composition of the dye will be assured, as more fully described hereinafter. In place of the log- 70 wood extract, as the vegetable dye-stuff to be employed, I may use other vegetable extracts such as those of cutch, quebracho, quercitron, etc., where other colors than shades of blue are desired in the dyed 75 product.

It is well known that dyewood extracts, especially logwood, are poorly soluble in cold water, are more soluble in hot water and are readily soluble with alkalis. It has here- 80 tofore not been found desirable to use solid extracts from these sources because of the expense of reducing the extract to the solid state as a commercial product, and because of the difficulty experienced by the dyer in 85 forming a solution from the said solid ex- tract when making up the dye bath. The standard liquid extracts of dyewoods are of a thick, syrupy and almost tarry consistency, which makes them troublesome and dis- 90 greeable to weigh or measure accurately in the dye-house, and it is one of the objects of my invention to permit the utilization of the dyewood extracts in a commercial form which will enable them to be readily handled 95 in the dye-house as well as be cheaply packed and shipped commercially.

I will now describe the preferred manner of making my improved dye composition, and by way of example I will employ log- 100 wood extract with the object of making a dye-stuff capable of producing a satisfac- 105 tory blue dye. I first provide an ammoniacal solution of hydrated cupric oxid which may be prepared by the mixture of blue stone, soda ash, and aqua ammonie, with or without an addition of water, and to this solution I add the requisite amount of liquid extract of logwood which produces a composition in a more or less dense condi- 110 tion (from paste to a dry powder, as preferred), which may be subsequently used

as a basis of the dye bath. More specifically, the said composition may be produced in the dried and powdered condition as follows:— To 50 grams of powdered blue stone, 50 grams of soda ash are added and thoroughly mixed; and to this dry mixture may be added 50 c. c. of strong commercial aqua ammonia 28%, with 20 c. c., more or less, of water to give a fluid. To one part by measure of this fluid, 6 parts of the liquid extract of logwood are added, and the mixture thoroughly stirred. The mixture will form a semi-solid mass which is then preferably dried and powdered. The drying should be performed by a natural evaporation, as the application of heat would be objectionable. It is to be kept in mind, that while the above proportions are given by way of example, I do not restrict myself thereto, as these proportions may be varied within considerable limits according to the special final condition of the product required. If, for example, 12 grams of the blue stone, 5 grams of soda ash, and  $3\frac{1}{2}$  c. c. of aqua ammonia 10%, were employed, and to one part of this solution 2 parts of the liquid extract of logwood  $51^{\circ}$  Twaddell is added, the resulting composition would be a thick pasty mass which may be packed and shipped in that form or dried to a powder, as preferred. In the forming of these solutions, the blue stone may first be dissolved in water and the soda ash dissolved in the aqua ammonia, and these solutions then mixed preliminary to the addition of the extract of logwood; such variations in the process being permissible, without altering the resultant composition, which is essentially a mixture including in its composition the extract of logwood and hydrated cupric oxid.

The solution to which the logwood is added is an ammoniacal solution of hydrated cupric oxid, and the proportions of the ingredients preferably employed are such that the soda ash and blue-stone (sulfate of copper) are in equivalent proportions, with the production of hydrated cupric oxid as a bulky carbonate precipitate; and when the above is supplemented by the addition of the aqua ammonia, said precipitate is dissolved and forms the ammoniacal solution of hydrated cupric oxid, a reagent which as far as I am aware has never heretofore been employed as a constituent in the dyeing of textile material.

The dye composition above described is in a form which enables the dyer to conveniently make up the dye liquor to be used in the dye-house, and hence this composition is especially advantageous owing to its convenient form, in addition to having the special quality of a permanent dye with capacity for direct dyeing. In giving the above examples, I have referred to the employment of blue-stone, but this is only as a

preferred salt where it is required to provide a blue dye from employment of logwood and it is to be understood that the metallic salt employed may be varied or supplemented by addition of other salts where the color or tint is to be varied. Similarly, the extract of logwood may be substituted by other vegetable dye substances such as cutch, sumac, quebracho, quercitron, etc., where other colors than blues are to be furnished. 75

If to the metallic and alkaline compounds above described by way of example, there be added to the solution (before mixing with the logwood) some pyrolignite of iron (say about 50 c. c.), the shade of blue will be deeper and toward a black. Furthermore, if a suitable proportion of bichromate of potash were substituted as part of the sulfate of copper in making up the ammoniacal solution of hydrated cupric oxid, the blue dye produced will be a deeper blue than when the sulfate of copper is the only metallic salt used. From these references to the additions to or substitutions of a portion of the main salt, it will be understood that my dye composition may be considerably varied, not only in producing different colors but in producing different shades of the same color. It is also to be kept in mind that the same metallic salt, such as sulfate of copper may be employed with the different vegetable dyes in producing the different colors, such as tans and browns, as well as the blues, but in cases where there is an extra quantity of tannin in the vegetable dye-stuff employed, it may be best to employ a salt of iron in place of that of copper, but I do not restrict myself in this substitution of the metallic salt nor to the specific use of any particular metallic salt. Similarly, I do not confine myself to the employment of logwood for the production only of the blue dye composition, as it may also be used for producing a reddish or wine color dye when employed with an ammoniacal solution of hydrated oxid with alumina or magnesia as the base, and these substances may be used in the commercial form of alum and Epsom salts respectively. 100

In the use of my improved dye composition, the same may be readily dissolved in water and employed as a single bath for dyeing the cotton, very much like the practice in respect to direct aniline dyes. By using soap or alizarin oil, or similar substances in the dye bath, the cotton may be entered dry, and thereby save time, trouble and expense which would otherwise be incident to the usual "wetting out" of the textile material before being placed in the dye bath. The use of soap has the advantage of cheapness, but the alizarin oil gives a brighter shade of the color. When the dye is made from logwood, as one of the constituents as hereinbefore described, the color pro- 115  
120  
125  
130

duced upon the cotton may be considered as a greenish-blue as it comes from the bath, but the blue color deepens on exposure to the air in the drying operation. The color 5 is imparted to the cotton fiber as a true dye and not as a precipitate, and consequently it is fast and moreover is so permanent that it will not "bleed" by subjecting the dyed garment to continued soaking in water.

10 While I prefer that the proportions of the sulfate of copper and the soda ash shall neutralize each other in the production of a bulky precipitate of the carbonate of copper which is to be dissolved by the ammonia added thereafter, the proportion of the soda ash used may provide a basic carbonate of copper if so desired. It is also to be understood that the cupric oxid of copper is not precipitated separately as metal oxid, but 15 through the formation of this oxid into a salt with the weak acid, carbonic acid, it is enabled to go into solution when the ammonia is added and thus aids in providing a true dye when the extract of logwood is introduced. While the dye mixture may be brought into a dry and powdered condition by its compounding, nevertheless the mixture is readily soluble in water and produces a true dye as distinguished from those 20 cases where a precipitate is held in suspension in the solution and deposited as a paste upon the textile material.

25 In this specification and claims, where I have referred to a metallic oxid, such as hydrated cupric oxid, etc., I do not restrict myself to a simple oxid of the metal, but intend to convey the meaning that my composition dye includes such a metallic oxid in association with the other substances 30 which enter into the composition of the compound; and moreover, that my ultimate composition as a dye will be modified according to the materials employed, as it will include whatever secondary substances may 35 be present owing to the particular wood dyestuff employed or the particular metallic and alkaline salts which may be employed in forming the dye, and I have therefore only referred to the more essential elements which 40 enter into the making of the composition such as the hydrated metallic oxid and the vegetable dyestuff, the ammonia being present as a vehicle for maintaining the resulting composition in a soluble form whereby 45 it forms a true dye as above stated.

50 I have described my invention in accordance with the general knowledge I have upon the subject resulting from the actual making and utilization of the dye composition 55 in the manner above described; and therefore while I have explained the manner of

the making of the dye composition and the utilization thereof in the process of dyeing, the foregoing specification is to be taken as a general exposition of the invention and 65 not as a limitation thereof in respect to minor results or compounds resulting from the complex inorganic reactions which may occur, an understanding of which is not material to the general essence of the invention. 70

Having now described my invention, what I claim as new and desire to secure by Letters Patent, is:—

1. As an article of manufacture, a dye composition in dried and powdered condition and comprising a vegetable dye extract and ammoniacal hydrated cupric oxid. 75

2. As an article of manufacture, a dye composition in dried and powdered condition containing an extract of logwood and 80 an ammoniacal hydrated metallic oxid.

3. As an article of manufacture, a dye composition in dry condition and containing an extract of a vegetable dye substance and 85 a hydrated oxid of a non-alkaline metal.

4. The herein described method of preparing a dye bath for dyeing cotton goods, which consists in first preparing an ammoniacal solution of hydrated oxid of a metal, then adding thereto a vegetable dye extract, 90 in proportion to produce a composition in a non-fluid condition.

5. The herein described method of preparing a dye for dyeing cotton goods, which consists in treating a mixture comprising a non-alkaline metallic salt and an alkaline salt with aqua ammonia in sufficient quantity to form an ammoniacal hydrated solution of an oxid of the non-alkaline metal and prevent a precipitate being 95 formed, mixing with the fluid compound so formed a vegetable dye extract to form a relatively thick pasty compound, and finally drying the same.

6. The herein described method of preparing a dye for dyeing cotton goods, which consists in mixing a non-alkaline metallic salt in powdered condition with an alkaline salt also in powdered condition, adding aqua ammonia to the mixture to dissolve it and forming an ammoniacal hydrated solution of an oxid of the non-alkaline metal, mixing with the fluid compound so formed a vegetable dye extract to form a relatively thick pasty mass, and finally drying the 110 compound. 115

In testimony of which invention, I hereunto set my hand.

JOHN W. FRIES.

Witnesses:

R. M. HUNTER,  
FLORENCE DEACON.